

## UNITED STATES PATENT OFFICE

GEORGE CHRISTOPHER MARRIS, OF LONDON, GEOFFREY RICHARD POLGREEN, OF WEMBLEY, AND STANLEY VAUGHAN WILLIAMS, OF KENTON, ENGLAND

## MANUFACTURE OF NICKEL IRON ALLOYS

No Drawing. Application filed December 16, 1930, Serial No. 502,848, and in Great Britain January 22, 1930.

This invention relates to the manufacture of nickel iron alloys in the form of powder, the object of the invention being the production of such powdered alloys in an improved manner whereby the alloyed powder produced has a particle-size distribution and other physical properties which render it suitable for the manufacture of cores for loading coils, electromagnets or the like.

10 A process for the production of nickel-iron powders is already known wherein the mixed oxides of the metals are reduced in a stream of gas. We have found that it is not easy by that process to obtain the alloy in a suitable physical state. If the reduction temperature is low, the metals do not alloy sufficiently rapidly; if it is high, though the alloying is complete, the grain size of the resulting powder is too large, and the particles are not easily broken up. We have found further that this difficulty can be removed by reducing at a low temperature and heating the reduced powder for a suitable time to a higher temperature, especially if 20 the reduced powder is washed before being raised to the higher temperature. The heating of the powder at the higher temperature generally results in the formation of a coherent block; it will therefore be termed 25 here sintering; but it must be understood that the aggregation of the particles is not an essential element of the process, and that the beneficial results of the second heating, which we term sintering, may be obtained 30 when the material remains a powder.

According to the first feature of the invention the manufacture of alloy powders containing nickel and iron by the reduction of the mixed oxides of the metals in a stream of gas comprises the sintering of the reduced powder at a temperature higher than that of reduction, whereby alloying is completed and a favourable size and physical character of the particles is produced. Preferably the reduced powder is washed in water or a dilute acid (for example dilute hydrochloric acid) after reduction and before sintering. If the particles of the reduced powder are already slightly sintered together, they should be broken up before washing.

The sintered material has now to be reduced to a fine powder, and then annealed to improve its magnetic properties. There is some danger that further sintering may occur during annealing and that the most suitable size and character of the particles, obtained after sintering and powdering, may be lost. According to a second feature of the invention, sintering during annealing is prevented by mixing the powder during annealing with a suitable quantity of a fine refractory powder. Preferably this refractory powder is mixed with the metal powder during the powdering of the metal after sintering. Talc is a suitable refractory powder.

Thus, in an example of one method of carrying out the process in accordance with the invention, suitable weights of nickel and iron oxides in powder form and in such proportions as to give the desired proportions of nickel and iron in the resulting alloy, are mixed together. The powders are mixed either in the dry condition by means of a mechanical mixer, or may be mixed in a wet condition by means of a mechanical mixer, or may be mixed in a wet condition by means of a colloid mill. If the latter alternative is adopted, the suspension is filtered after mixing and is then dried.

The mixed oxides are now reduced in a current of hydrogen at a suitable temperature, (850° for example). The product of reduction may now be in a slightly sintered condition, but can be readily broken down to a fine powder in a rotary pulverizer.

The fine product is now washed with a five per cent hydrochloric acid solution at 50° C., one litre of solution being allowed for each kilogram of alloy. The acid is next decanted, and the powder is washed thoroughly with cold water and dried in an oven.

The washed powder is now sintered by heating it to a higher temperature (about 1,000° C.) in a reducing atmosphere for about one hour, and is then allowed to cool slowly to room temperature. It is next broken up in a pulverizer, and is then ball-milled to give smooth, even particles. Where a large particle size is required, the sintering is car-

ried out at a higher temperature, and vice versa.

The metal powder is now mixed with about 2½% of fine talc powder and annealed.

- 5 If the metal is a 80:20 nickel iron alloy, it may be annealed at about 900° C. It is then provided with a suitable insulating coating and pressed into cores. The coating may suitably be produced by heating the powder in a solution of chromic anhydride and a halogen acid or halogen salt, the heating being continued until the solution has evaporated substantially to dryness.

10 The process in accordance with the invention may conveniently be applied to magnetic alloys containing nickel, iron and cobalt, such as the known ternary alloys in which these elements are used to give the required magnetic qualities, low hysteresis loss, for example.

15 What we claim is:—

1. A process for the manufacture of alloy powders containing nickel and iron, which comprises mixing the powdered oxides of nickel and iron, reducing the mixture by heating in a reducing gas, washing the product, drying the product, and sintering the product at a temperature higher than the temperature used for the reduction of the mixture.

2. A process for the manufacture of alloy powders containing nickel and iron, which comprises mixing the powdered oxides of nickel and iron, reducing the mixture by heating in a reducing gas, washing the product, drying and sintering the product at a temperature higher than the temperature used for the reduction of the mixture, and then subjecting the mixture to pulverization.

3. A process for the manufacture of alloy powders containing nickel and iron, which comprises mixing the powdered oxides of nickel and iron, reducing the mixture by heating in a reducing gas, washing the product, drying and sintering the product at a temperature higher than the temperature used for the reduction of the mixture, pulverizing the product, mixing the pulverized product with a refractory powder and annealing the resultant mixture.

4. A process for the manufacture of alloy powders containing nickel and iron, which comprises mixing the powdered oxides of nickel and iron, reducing the mixture by heating in a reducing gas, washing the product, drying and sintering the product at a temperature higher than the temperature used for the reduction of the mixture, pulverizing the product, mixing the pulverized product with powdered talc, and annealing the resultant mixture.

5. A process for the manufacture of alloy powders containing nickel and iron, which comprises mixing the powdered oxides of nickel and iron, reducing the mixture by

heating in a reducing gas, washing the product, drying and sintering the product at a temperature higher than the temperature used for the reduction of the mixture, pulverizing the product, mixing the pulverized product with a refractory powder, annealing the resulting mixture and then coating the metal particles with an insulating coating.

6. A process for the manufacture of alloy powders containing nickel, iron and cobalt, which comprises mixing the powdered oxides of nickel, iron and cobalt, reducing the mixture by heating in a reducing gas, washing the product, drying and sintering the product at a temperature higher than the temperature used for reducing the mixed oxides.

7. Cores for loading coils and electromagnets comprising a nickel iron alloy pressed from powdered alloy obtained by reducing a mixture containing nickel oxide and iron oxide by heating in a reducing gas, sintering the product at a temperature higher than that used for the reduction, pulverizing the sintered alloy and coating the alloy particles with an insulating coating.

95 GEORGE CHRISTOPHER MARRIS.

96 GEOFFREY RICHARD POLGREEN.

97 STANLEY VAUGHAN WILLIAMS.

98

100

105

110

115

120

125

130